

Sept. 3, 1968

H. K. NIELSEN, JR., ETAL

3,400,043

PROCESS OF ADDING BITUMINOUS ADDITIVES TO A FIBROUS  
MATERIAL IN THE GRINDING ZONE OF A REFINER

Filed June 1, 1964

2 Sheets-Sheet 1

Fig. 1.



Fig. 2.

INVENTORS

HANS K. NIELSEN, JR.  
DAVID E. NOYES  
GILBERT GODIN  
FRED C. NORRARD

*John G. McNamee*  
ATTORNEY

Sept. 3, 1968

H. K. NIELSEN, JR., ET AL. 3,400,043

PROCESS OF ADDING BITUMINOUS ADDITIVES TO A FIBROUS

MATERIAL IN THE GRINDING ZONE OF A REFINER

Filed June 1, 1964

2 Sheets-Sheet 2



INVENTORS

HANS K. NIELSEN, JR.  
DAVID E. NOYES  
GILBERT GODIN  
FRED C. NORSGARD

*John A. McNamee*  
ATTORNEY

1

3,400,043

**PROCESS OF ADDING BITUMINOUS ADDITIVES TO A FIBROUS MATERIAL IN THE GRINDING ZONE OF A REFINER**

Hans K. Nielsen, Jr., Dunellen, David E. Noyes, Somerville, Gilbert Godin, Millington, and Fred C. Norgard, Somerville, N.J., assignors to Johns-Manville Corporation, New York, N.Y., a corporation of New York

Filed June 1, 1964, Ser. No. 371,678  
8 Claims. (Cl. 162—171)

**ABSTRACT OF THE DISCLOSURE**

A fibrous aqueous mixture is introduced to the grinding zone of a refiner, and fluid bituminous material, e.g., asphalt, having a melting point higher than the temperature of the mixture, is introduced into the mixture in the grinding zone and cooled and solidified and intimately mixed with the mixture, without clogging of the refiner.

This invention relates to the manufacture of lignocellulosic fiber and to products containing such fiber. More particularly, the invention relates to a process for introducing molten additives to fibrous material as it is being ground and refined in preparation for manufacture of fibrous products.

In the manufacture of fiber board, it has long been common practice to incorporate additives with the fibrous material in order to impart certain desired properties to the final product. In many cases, this does not cause any processing difficulties, as various types of additives may be introduced directly into the fiber refining apparatus, or may be added to the pulp after the refining operation and prior to the felting operation. Some products, however, require the addition of normally solid, thermoplastic substances for waterproofing, strengthening, or other purposes. Addition of these materials, such as, for example, asphalt or other bituminous substances, has been the subject of a great deal of development work over the years, which has resulted in several generally accepted methods of material introduction.

One method of incorporating bituminous material in fibrous stock is to introduce it in the form of dry particles to the refining apparatus, or to mix it with the fibrous slurry after the pulp has been formed. While a satisfactory board product can be made from such slurries, poor retention and nonuniform distribution of the bitumen often occur. Grinding of the bitumen is often required, increasing the cost of the process. The type of bitumen utilized must have a relatively low penetration value, to permit storage without coalescence of the particles, while at the same time possessing a low enough softening point so that the material melts in the drier. Such material can be obtained from only a limited number of sources and is relatively expensive.

Bituminous material is also introduced to pulp slurries in the form of an emulsion, which requires use of emulsifying agents in addition to a colloidizing operation. Storage of the bituminous material is a problem with this system, as in the dry particle method mentioned in the previous paragraph. Boards containing bitumen introduced in this manner are subject to problems of intermittent bitumen coverage and poor retention. In addition, the amount of emulsion which can be used is limited because it slows the drainage time of the fibrous stock a considerable amount.

It has been suggested to introduce bituminous material in its molten form, either to the fibrous slurry after it has been formed and just prior to its introduction to a board forming machine, or to the beating or mixing apparatus along with the fibrous material and water. Introduction of

2

molten bitumen to an aqueous slurry of fibers is described in U.S. Patent No. 3,087,851. But this arrangement requires special apparatus for introducing the molten asphalt to the slurry, and furthermore, an additional refining operation is provided prior to sending the stock to the board forming machine.

Fluid bitumens have been introduced directly to a beater or mixer at the same time that fibers and water are introduced, as disclosed in U.S. Patents Nos. 1,449,221, 1,844,951, and 1,878,300. According to the processes described in these patents, however, the fluid bitumen is mixed with hot water and cellulosic material, and the mixture is maintained at a temperature in the mixer such that the bituminous material remains in its fluid or nonsolid state. The fibrous material removed from the mixing apparatus is coated with the bitumen, and may be felted or molded into a product in the usual manner. This operation takes a relatively long time, however, due to the necessity of thoroughly mixing the materials to ensure coated fibers. In addition, it does not lend itself to providing a fibrous slurry containing small, discrete bitumen particles intermixed with the fibers. This type of stock is preferred in fiberboard manufacture because the drainage time is faster than that of stock containing bitumen coated fibers. The bitumen in such stock becomes thoroughly mixed with the fibers in the final product, since at the end of the felting operation, the wet fibrous mat is dried at temperatures which melt the bitumen particles, permitting the fluid bitumen to flow and homogeneously pervade the fibrous material.

U.S. Patent No. 2,402,160 describes the process of introducing molten asphalt directly into a refining apparatus specifically described as an Asplund defibrator. This type of refiner includes a steam chest into which slightly moist wood chips are introduced. The lignin in the wood chips, binding the fibers together, is plasticized to such an extent that the fibers are readily sheared apart with a minimum of cutting. Liquid asphalt is forced into the preheater of the apparatus where it mixes with the wood being fed to the grinding discs, and the grinding action in the grinding zone is carried out while the asphalt is maintained as a liquid, resulting in asphalt coated fibers being discharged from the machine.

The manner of introducing asphalt in the Asplund defibrator cannot be extended to refiners such as the Bauer, Sprout-Waldron, or Allis-Chalmers mills or refiners, since such apparatus does not operate in the same manner as the Asplund defibrator. The Bauer refiner, and other apparatus of the same general type, is comprised generally of two ribbed discs rotating in opposite directions, or one rotatable disc working against a stationary plate or disc, to which discs treated wood chips, pulp, or raw wood, in the presence of a substantial amount of water, are fed. The material is subjected to a rubbing and partial cutting action as it passes between the ribbed surfaces of the discs toward the peripheries thereof under centrifugal forces produced by the rapid rotation. Since the water introduced to the Bauer is much cooler than molten asphalt or other molten bitumens, introduction of molten asphalt to the mixture of wood and water would cause the asphalt to agglomerate upon contact with the water, before the mixture was subjected to the grinding and refining action of the discs. This would cause an almost immediate clogging of the system. It is recognized that Patent No. 2,402,160 discloses that the coated fiber discharged from the Asplund defibrator may be mixed with water and further refined in a Bauer refiner, but this is possible because the asphalt will already have been thoroughly mixed with the wood fiber and is present only as a relatively thin coating on the fibers. Moreover, the asphalt is combined with only a small amount of water prior to being introduced into the Bauer refiner.

Notwithstanding the years of efforts of the fiberboard industry to find a way to introduce bituminous materials efficiently and inexpensively into a fibrous slurry, and to obtain a high quality, uniform product, there has been no method known to the present inventors for introducing molten asphalt directly to the grinding zone of a refiner and obtaining a fibrous slurry containing uniformly distributed asphalt particles.

It is an object of the present invention to provide a novel process for introducing molten asphalt, or other normally solid, thermoplastic material, to a refiner without heating the grinding chamber, or the fibrous mixture fed thereto, to maintain the asphalt in a fluid state.

It is another object of the invention to provide a process for introducing molten asphalt, or other normally solid, thermoplastic material, to a refiner without having to mix the asphalt with fibrous material and water prior to such introduction.

Another object of the invention is to provide a process for introducing molten asphalt, or other normally solid, thermoplastic material, to a refiner which requires only a slight modification of existing refiner structures.

Briefly, the invention comprises introducing an aqueous mixture containing fibrous material to the grinding zone of a refiner apparatus, the zone comprising grinding surfaces, one rotating with respect to another, and introducing fluid thermoplastic material directly to the grinding zone where, surprisingly, it does not agglomerate and clog the apparatus but is thoroughly intermingled with the aqueous mixture. The melting point of the thermoplastic material is higher than the temperature of the aqueous mixture, whereby the thermoplastic material cools and solidifies upon contact with the aqueous material. By grinding the fibrous material and the solidified thermoplastic material together, the materials are intimately mixed.

The nature of the invention will be more fully understood and other objects may become apparent when the following detailed description is considered in connection with the accompanying drawing, wherein:

FIG. 1 is a simplified flow diagram of a refining operation;

FIG. 2 is a pictorial representation of a rotary disc refiner;

FIG. 3 is a sectional view taken on the longitudinal axis of the grinding chamber of the rotary disc refiner of FIG. 2;

FIG. 4 is a front elevational view of the grinding face of an open grinding head or disc; and

FIG. 5 is a partial sectional view taken on the longitudinal axis of spaced grinding discs, and showing a modified means for introducing thermoplastic material to the grinding zone.

Referring to the drawings, a typical flow diagram of a fiberboard manufacturing process is illustrated in FIG. 1. Wood chips are stored in a bin or silo 10 and are introduced with a predetermined amount of water to a primary refiner 12, such as, for example, a Bauer refiner. The wood is defiberized in the refiner and the resulting pulp is delivered to a refiner chest 14, from which it is then fed to a regulator 20, where pulp of the proper consistency is permitted to pass through a proportioner 22 and then to a machine chest 24. The pulp or slurry in the machine chest may be introduced to a board forming machine, such as a Fourdrinier machine, where it is formed into a wet mat of fibers and subsequently dried to form a fiberboard product.

The process steps described thus far are well known in the art. The process made possible by the present invention contemplates the additional step of adding a molten thermoplastic material, such as asphalt, to the wood chips and water in the refiner. This requires a source of molten asphalt 26, which is generally more available and inexpensive than the type of asphalt employed when mixed in its dry state. Use of molten asphalt eliminates the need

for granulating and milling dry asphalt, and also eliminates the storage problems associated with the use of dry asphalt.

As previously explained, one refining apparatus to which this invention is applicable is that which incorporates grinding discs, such as in a Bauer refiner. In FIG. 2, a typical Bauer refiner 30 is illustrated as having a base support 32 on which are mounted two spaced motors 34 and 36. Shafts 38 and 40, connected to motors 34 and 36, respectively, rotate in opposite directions and extend into a disc housing or casing 42 mounted between the motors. A wood delivery chute 44 communicating with a source of wood chips (not shown) is connected to the upper portion of the casing 42 to permit fibrous material and water to be introduced into the grinding zone, as will be explained in more detail hereinafter.

Referring now to FIGS. 3 and 4, the end of shaft 38 carries an open head or disc 50, and the end of shaft 40 carries a closed head or disc 52. The central portions of the discs are frusto-conical in shape, with their convex sides or faces directed away from the delivery chute 44, and are spaced from each other, thereby defining a grinding zone or chamber 54 therebetween. The discs have opposed peripheral portions 56 and 58 to which cutting and grinding rings 60 and 62 are attached, as by bolts 64. Each ring is provided with ribs or blades 66 for grinding wood chips fed to the refiner.

As best shown in FIG. 4, the frusto-conical portion of open head 50 is provided with three equispaced apertures 68 in order to admit wood and water into the grinding zone between the discs. As shown in FIG. 3, a flanged ring 70 having apertures therein corresponding to the apertures 68 is attached to the concave side of the open head 50 and is so arranged that the annular flange 72 thereof extends adjacent the upper portion of the delivery chute outlet 74, defining with plate 75 an inlet chamber 76. Above the flange 72 and with the inlet chamber 76, a hollow plug wiper 79 is disposed so that its extremity is adjacent the open head 50. The conduit 81 in the plug wiper 79 normally is connected to a source of water.

The operation of the standard equipment thus far described is as follows. Wood chips are metered into the chute 44 by a metering wheel 78, and water is sprayed from tubes 80 to mix with the falling chips. The mixture of chips and water moves into the inlet chamber 76, through the openings or apertures 68 in the open head 50, and into the grinding zone 54. Most of the mixture will pass through the openings 68 disposed adjacent the upper half of the inlet chamber, but chips and water falling below the shaft 38 are directed by the sloped flange 72 toward an opening 68 adjacent the lower half of the inlet chamber, through which it can pass into the grinding zone 54. The mixture is hurled toward the grinding rings 60 and 62 by the centrifugal force of the rotating discs, and then passes between the ribbed rings. The wood chips are finely ground and pulped during passage through the rotating rings, and the resulting fibrous slurry drops through an opening at the bottom of the housing 42 directly to the refiner chest or to an intermediate storage vessel from which it is pumped to the chest. Should any buildup of fiber occur on the open head 50, it will be wiped therefrom by the plug wiper 79 which, as previously stated, is mounted closely adjacent to the head 50. Further cleaning of the head and the apertures 68 is obtained by spraying water through the conduit 81. Although not shown, additional water may be introduced to the grinding zone by sprays from within the housing 42.

It has been found that molten thermoplastic material can be successfully introduced directly into the refiner if it is cooled and maintained in nonmolten condition in the grinding zone. This may be accomplished by spraying the molten material substantially directly into the grinding zone, so that little, if any, molten material is mixed with the mixture of water and wood chips before

entering the grinding zone. When molten asphalt, for example, is introduced into the grinding zone in this manner, it experiences a thermal shock; that is, there is an immediate heat transfer as the material contacts the water. Drops of the asphalt spray solidify upon suddenly cooling and tend to crack or fracture into smaller solid particles. In addition, such particles are subjected to mechanical attrition as they pass between the grinding discs. In this manner, the molten asphalt is converted to small particles of solid asphalt in the grinding zone of the refiner, and the small asphalt particles are intimately mixed with the wood fibers. If the molten asphalt were introduced to the mixture of wood chips and water in the feed chute 44, it would tend to agglomerate and clog the apparatus. It can be introduced in the inlet chamber 76 at a location spaced from the open disc 50, however, so long as the velocity of the asphalt droplets is enough to carry them into the grinding zone before they solidify or, if solidification begins before the droplets are entirely within the grinding zone, so long as the velocity of the droplets is enough to carry them into the grinding zone without agglomerating in the inlet chamber of the apparatus.

A practical means of carrying out the method of this invention is to connect the conduit 81 of the plug wiper 79 to a source of molten asphalt, or to provide another molten asphalt nozzle such as indicated at 82 in FIG. 3. By locating the asphalt spray nozzle close to the open disc 50, substantially all of the molten asphalt first contacts the mixture of water and cellulosic material in the grinding zone 54, or just prior to entering the zone, and does not agglomerate in the inlet chamber. The small amount of asphalt that accumulates on the land portions between the openings 68 in the open disc 50 is scraped therefrom by the wiper 79, and this material, upon being thrown into contact with the incoming mixture of water and chips by the rotation of the open disc 50, is carried by the mixture into the grinding zone where it is refined into small particles.

Several variables relating to the specific materials utilized and to the operating requirements of the equipment must be considered. In order to introduce asphalt in its fluid state to the refiner, it must be heated to a temperature which exceeds its melting point by an amount sufficient to cause it to be fluidized. Also, the viscosity of the asphalt must be such as to permit it to be pumped. In order to maintain the required temperature and viscosity of the asphalt, it is desirable to pump it to the refiner through a heated pipe.

The temperature of the mixture of chips and water introduced to the refiner preferably is ambient, but it may vary considerably according to the temperature and type of asphalt. In order to effect a heat transfer sufficient to suddenly cool and solidify the asphalt, the mixture should be cooler than the melting point of the asphalt and be present in sufficient amount to effect such transfer. In order to ensure proper flow, the asphalt is preferably heated to a temperature well above its melting point and, because it is exposed to the fibrous slurry mixture for only a relatively short time, in the order of 1 to 2 seconds, the temperature of the mixture is preferred to be substantially lower than that of the asphalt.

As stated previously, it is preferred that the outlet of the nozzle spray be closely spaced from the rotating open head, as, for example, about  $\frac{1}{4}$  inch away. The asphalt should be sprayed at sufficient velocity to preclude asphalt droplets from falling to the bottom of the inlet chamber and agglomerating there. The nozzle outlet may be moved closer or farther away from the head, so long as the combination of the spray velocity and distance from the grinding zone are such as to prevent the asphalt from solidifying and agglomerating in the inlet chamber.

It is to be understood that there are methods of introducing asphalt to the grinding zone other than by spacing

a nozzle from an open grinding head. Referring to FIG. 5, discs 50 and 52 are mounted on shafts 84 and 40, respectively, as in the arrangement of FIG. 3. Instead of a separate asphalt spray nozzle, however, a conduit 86 is provided in the shaft 84, the conduit terminating at 88 in the grinding zone between the two discs. Thus, with this arrangement, molten asphalt can be introduced to the grinding zone through the conduit 86, thus eliminating the chance of asphalt agglomeration outside of the grinding zone.

The following examples illustrate various combinations of asphalt and water fed to a Bauer refiner under different conditions, all resulting in an intimate mixture of asphalt particles and wet fibers. In the physical arrangement for the introduction of asphalt in the examples given, a nozzle was located in the inlet chamber, and was spaced about  $\frac{1}{4}$  inch from the open head or disc.

| Example                              | I             | II            | III           |
|--------------------------------------|---------------|---------------|---------------|
| Asphalt:                             |               |               |               |
| M.P., ° F.                           | 190           | 210           | 250           |
| Temp., ° F.                          | 375           | 400           | 450           |
| Gal. per min.                        | 0.1-5         | 0.1-5         | 0.1-5         |
| Viscosity, SF at 400° F. (max.)      | 125           | 125           | 125           |
| Water:                               |               |               |               |
| Temp., ° F.                          | 70-140        | 70-140        | 70-140        |
| Gal. per min.                        | 2-6           | 2-6           | 2-6           |
| Size of asphalt spray nozzle, inches | $\frac{1}{4}$ | $\frac{1}{4}$ | $\frac{1}{4}$ |

In practice, the type of asphalt or other thermoplastic material utilized depends upon the end use of the fibrous product and the temperature of the ovens used to dry the felted or molded product. Where the fibrous mixture is to be felted on a board-making machine, the asphalt added to the mixture generally has a softening point in the range of about 150° F. to 300° F. Asphalt has been added in amounts as high as 80% of the stock mixture, based on the total dry weight of solids and asphalt. The 80% amount is by no means the maximum amount of asphalt which can be added, however, since at that level, there was no indication that a peak was being reached.

As mentioned previously, this invention is not limited to the specific disc refiner discussed, but may be practiced on modified arrangements, such as refiners employing a single rotating disc in combination with a fixed plate or disc. It is not necessary that the invention be limited to a disc type of refiner, since it could well be practiced on a plug type refiner, for example. Basic equipment requirements are a means for introducing molten asphalt directly into the grinding zone of a refiner, and solidifying and grinding the asphalt in the grinding zone.

While the invention has been described particularly with respect to the addition of asphalt to a fibrous mixture, it should be understood that any suitable thermoplastic material whose melting point is higher than the temperature of the water and chips introduced to the refiner can be used.

It is to be understood that variations and modifications of the present invention may be made without departing from the spirit of the invention. It also is to be understood that the scope of the invention is not to be interpreted as limited to the specific embodiments disclosed herein, but only in accordance with the appended claims, when read in the light of the foregoing disclosure.

What we claim is:

1. A process for producing fibrous material intimately mixed with a bituminous material, comprising the steps of:
    - (a) introducing an aqueous mixture containing fibrous material to the grinding zone of a refiner apparatus, the zone comprising grinding surfaces, one rotating with respect to another,
    - (b) introducing molten fluid bituminous material into the grinding zone,
- the temperature of the aqueous mixture is wherein lower than the melting point of the bituminous material and thereby causing the bituminous material to solidify in the grinding zone.

- (c) maintaining the bituminous material in solid condition in the grinding zone, and
  - (d) grinding the fibrous material and the solidified bituminous material together to intimately mix the same.
2. A process for producing fibrous material is recited in claim 1, wherein the bituminous material is asphalt.
3. A process for producing fibrous material as recited in claim 2, wherein substantially all the asphalt is in molten condition as it enters the grinding zone.
4. In the process of refining fibrous material in a refining apparatus comprising a grinding zone and a connecting material inlet chamber, the grinding zone comprising relatively rotating grinding surfaces moving at high speeds, the improvement comprising the steps of:
- (a) introducing an aqueous mixture of relatively large pieces of fibrous material to the inlet chamber,
  - (b) moving the aqueous mixture into the grinding zone,
  - (c) introducing molten fluid bituminous material substantially directly to the grinding zone,
- wherein the temperature of the aqueous mixture is substantially cooler than the temperature of the bituminous material and the melting point thereof,
- (d) mixing the aqueous mixture and the bituminous material in the grinding zone a sufficient length of time to solidify the bituminous material, and
  - (e) grinding the fibrous material and the solidified bituminous material between the grinding surfaces to intimately mix the two materials.
5. A process of refining fibrous material as recited in claim 4, wherein the bituminous material is asphalt having a melting point in the range of about 150° F. to about 300° F.
6. A process of refining fibrous material, comprising the steps of:
- (a) introducing an aqueous mixture of fibrous material to a grinding zone comprising relatively rotating grinder surfaces in a housing,
  - (b) introducing molten fluid bituminous material to the grinding zone in spray form,
- wherein the temperature of the aqueous mixture is substantially less than the melting point of the bituminous material, whereby the droplets of the spray of bituminous material cool and solidify upon contact with the aqueous mixture,

- 8
- (c) grinding the fibrous material and the solidified bituminous material between the relatively rotating grinding surfaces in the housing,
  - (d) and discharging the ground and mixed fibrous material and bituminous material from the housing.
7. In a process of refining fibrous material in a refining apparatus having:
- (a) oppositely facing grinding discs spaced apart at their central portions and in grinding relationship at their outer portions,
  - (b) the space between the grinding discs comprising a grinding chamber, and
  - (c) an inlet chamber communicating with the grinding chamber,
- the steps of:
- (d) introducing an aqueous mixture of cellulosic material to the inlet chamber,
  - (e) moving the mixture into the grinding chamber,
  - (f) introducing molten fluid bituminous material into the grinding chamber substantially without contact with the aqueous mixture in the inlet chamber,
- wherein the temperature of the aqueous mixture is considerably lower than the melting point of the bituminous material,
- (g) mixing the aqueous mixture with the bituminous material for a relatively short period of time, but long enough to cause the bituminous material to cool and solidify, and
  - (h) moving the aqueous mixture and the solidified bituminous material outwardly from the grinding chamber between the grinding surfaces of the discs, whereby the cellulosic material and the solidified bituminous material are ground and intimately mixed together and discharged from the grinding chamber.
8. A process of refining fibrous material as recited in claim 7, wherein the bituminous material is sprayed into the grinding chamber.

#### References Cited

##### UNITED STATES PATENTS

|           |        |                 |       |         |
|-----------|--------|-----------------|-------|---------|
| 2,402,160 | 6/1946 | Heritage        | ----- | 162—10  |
| 3,087,851 | 4/1963 | Beuscher et al. | ----- | 162—171 |

S. LEON BASHORE, Primary Examiner.

R. BAJEFSKY, Assistant Examiner.